

# UNITED STATES PATENT OFFICE

JAMES SCOTT, OF HAMILTON, CANADA.

## IMPROVEMENT IN COMPOSITIONS FOR ELASTIC STAMPS.

Specification forming part of Letters Patent No. **167,856**, dated September 21, 1875; application filed June 12, 1875.

*To all whom it may concern:*

Be it known that I, JAMES SCOTT, of the city of Hamilton, in the county of Wentworth, in the Province of Ontario, Dominion of Canada, have invented a new and useful Improvement in Compounds for Composition Stamps; and I do hereby declare that the following is a full, clear, and exact description of the construction and operation of the same.

The invention relates to that class of compounds of which yielding stamps are made for ornamenting sewing or other machines with bronze, gold-leaf, silver-leaf, &c.

It has been found that yielding or pliable composition stamps are affected by cold, and in winter will only last, on an average, about three weeks, and in warm weather a little longer. The fine lines of the stamps lose their sharpness, and the spaces between the lines become filled up, so as to deface the pattern and render a perfect impression an impossibility. When the stamps are in this condition, from two to three weeks' usage, they are obliged to be thrown away as entirely useless, and other stamps formed of new material.

It will be seen that the stamps, in the first place, do not last long, and that when they are worn out they are thrown aside as useless; whereas I have used my stamps during last winter for three months, and at the end of that time they were not worn out, but were almost as good as new. When they are worn out I can easily remold them, either in the original pattern or a different pattern.

It will be observed that, in the first place, my stamps are not affected by cold, they stand wear much longer than the present ones, and are more quickly and cheaply made, and a great saving over the old ones, as there is no waste, every stamp being capable of being remolded.

To prepare the stamps, I take gelatine and put it in a water-bath until it is soaked to the thickness of a knife-blade; then I prepare

it for boiling in a glue-pot or other suitable vessel, and dissolve it. In about twenty minutes' time I add to it about four (4) ounces of glycerine, and one (1) pound of glue, and two table-spoonfuls of the best sirup, and about one-tenth of an ounce of tannin; stir five minutes to thoroughly mix. The compound is then formed into a plaster-of-paris or lead mold, (having the desired design impressed therein from a prepared or cut block of wood or metal,) where it remains for about two hours. When it is taken out it solidifies and is ready for use in the usual manner of ornamenting with the old stamps.

When my stamps are worn out, which is not until three months' constant use, I place them in a warm bath for about one minute; then take them out and scrape out the outside, which removes the old varnish; then put them into a water-bath and dissolve. When the substance becomes about the consistency of thick sirup it is poured into a plaster-of-paris or metal mold, and in a very short time is again ready for use.

Many attempts to remold old worn-out stamps have been made by others, but hitherto without success.

It will be observed that I do not claim to be the first inventor of composition stamps or printers' ink-rollers, the basis of which is glycerine, glue, sugar, sirup, &c., as now used; but

What I do claim as new, and desire to secure by Letters Patent, is—

An improved compound for composition stamps for ornamenting with bronze, gold-leaf, and silver-leaf, consisting of gelatine, sirup, glycerine, in combination with tannin, substantially as and for the purpose specified.

Dated at Hamilton, Ontario, this 9th day of April, A. D. 1875.

JAMES SCOTT.

Signed in the presence of—

W.M. BRUCE,  
P. L. SCRIVEN.